

## UNITED STATES PATENT OFFICE.

GUSTAV PETZOLD AND HEINRICH RITTNER, OF OFFENBACH-ON-THE-MAIN, GERMANY,  
ASSIGNORS TO I. G. FARBENINDUSTRIE AKTIENGESELLSCHAFT, OF FRANKFORT-  
ON-THE-MAIN, GERMANY.

PROCESS OF PRODUCING COMBINED SHADES ON THE VEGETABLE FIBER AND IN  
MATERIALS TREATED ACCORDING TO SUCH PROCESS.

No Drawing. Application filed December 15, 1924, Serial No. 756,049, and in Germany January 29, 1924.

Our invention relates to a process of producing combined shades of azodyestuffs and vat dyestuffs on the vegetable fiber consisting in producing an azodyestuff according to one of the usual methods on the fiber. 5 an ester-salt of the leuco-compound of a vat dyestuff being present simultaneously, and in subjecting the goods to be dyed, to a treatment with oxidizing agents in an acid medium. The process may be conducted in such a manner, that the fiber is impregnated with a mixture of an aromatic nitrosamin-alkali-salt and an alkali-salt of an azo-component and an ester-salt of the leuco compound of a vat dyestuff and the dyestuffs are developed by treatment with oxidizing agents in an acid medium, or the fiber may be impregnated with an alkaline solution of an azo-component and developed with a diazo solution by adding an ester-salt of the leuco-compound of a vat dyestuff to the padding- or diazosolution and the goods to be dyed may be treated with oxidizing agents in an acid medium. Our invention 25 also relates to the product of such process.

Ester-salts of the leuco-compounds of vat dyestuffs, which are prepared by transforming leuco compounds of vat dyestuffs into acid esters of a polybasic acid, are described in the U. S. A. Letters Patent No. 1,448,251 of Marcel Bader and Charles Sunder, dated Mar. 13, 1923.

Mixtures of aromatic nitrosamin-alkali-salts and alkalisalts of certain azo components, some of which are on the market under the name of rapid-fast-colors, are described in the U. S. A. Letters Patent No. 1,193,566 of Felix Kunert, dated Aug. 8, 1916, and the application Serial No. 717,211 of Arthur Zitscher, filed June 2, 1924.

Our invention may be used for dyeing as well as for printing, yielding excellently fast combined colors of different shades, which were not known hitherto, and making it possible to supply the consumer with highly concentrated products immediately ready for use by simple operations.

In order to illustrate the new process

more fully the following examples are given. 50

## EXAMPLE 1.

The unprepared goods are printed with the following printing-color:

70 gr. of a paste of the nitrosamin-salt 55  
of 5-nitro-1,2-anisidin, corresponding to 23% of the base are  
mixed with  
10 gr. of caustic soda solution of 36° Bé. 60  
and  
70 gr. of water and poured in  
500 gr. of a neutral tragacanth thickening and then the following solution is added:  
20 gr. of  $\beta$ -naphthol in 65  
25. gr. of caustic soda solution of 36° Bé.  
and  
85 gr. of water and  
10 gr. of the product, prepared from indigo according to the U. S. A. 70 Letters Patent No. 1,448,251, dissolved in  
210 gr. of water are added and the whole  
is made up to

75

1000 gr.

The goods are dried, steamed for a short while and passed into a lukewarm to boiling bath, containing 25 to 30 gr. of sodium bisulfate, 30 to 40 cc. of a solution of nitrate 80 of iron of 20° Bé. in the liter rinsed, soaped and dried.

A brown is obtained.

## EXAMPLE 2.

The unprepared goods are printed with the following printing-color:

92 gr. of a paste, prepared from the 3-methyl-1-phenyl-5-pyrazolone sodium-salt and the nitrosamin-sodium-salt of 3-nitro-1,4-toluidin, corresponding to 16, 3% of the base, are mixed with  
200 gr. of cold water, poured in  
500 gr. of a neutral tragacanth thickening 95  
and then

10 gr. of the product, prepared from indigo according to the U. S. A. Letters Patent No. 1,448,251, dissolved in

198 gr. of water, are added and the whole is made up to

1000 gr.

The goods are dried, steamed for a short while and passed into a developing-bath such as described in connection with Example 1, or containing other similarly acting oxidizing agents, rinsed, soaped and dried.

15 A yellowish olive is obtained.

#### EXAMPLE 3.

The unprepared goods are printed with the following printing-color:

20 60 gr. of a paste, prepared from the sodium-salt of acetoacetyl-para-anisidin and the nitrosamin-sodium-salt of ortho-nitroanilin, corresponding to 21, 1%, of the base, are mixed with

25 200 gr. of cold water and poured in  
500 gr. of a neutral tragacanth thickening and then

30 10 gr. of the product, prepared from indigo according to the U. S. A. Letters Patent No. 1,448,251, dissolved in

35 230 gr. of water, are added and the whole is made up to

1000 gr.

The goods are dried, steamed for a short while and passed into the above mentioned developing-bath, rinsed, soaped and dried.

40 A greenish olive is obtained.

#### EXAMPLE 4.

##### Printing-color for green.

45 100 gr. of a paste, containing 15% of diacetoacetyl-ortho-tolidin, the nitrosamin-alkali-salt of 2,5-dichloroanilin and free caustic soda solution, are stirred with

50 200 gr. of cold water and poured in  
500 gr. of neutral tragacanth thickening, then

55 20 gr. of the product, prepared from indigo according to the U. S. A. Letters Patent No. 1,448,251, dissolved in

180 gr. of the water, are added and the whole is made up to

60 1000 gr.

The unprepared goods are printed with this printing-color, dried, steamed in acetic acid for 2 minutes, then passed into the above mentioned developing-bath, rinsed, soaped and rinsed once more,

In this manner beautiful green shades of an excellent fastness are obtained.

By using 20 gr. of the product, prepared from dibromindigo according to the U. S. A. Letters Patent No. 1,448,251, for the printing-color, a little more yellowish shades of a greater clearness are obtained.

#### EXAMPLE 5.

##### Printing-color for light-brown.

100 gr. of a paste, containing 15% of the anilid of 2,3-hydroxynaphthoic acid, the nitrosamin-alkali-salt of ortho-nitroanilin and free caustic soda solution, are stirred with

200 gr. of cold water and poured in  
500 gr. of neutral tragacanth thickening, then

10 gr. of the product, prepared from indigo according to the U. S. A. Letters Patent No. 1,448,251, dissolved in

190 gr. of water, are added and the whole is made up to

1000 gr.

The goods are printed with this printing-color in the same manner, as described in Example 1, dried, steamed in acetic acid, passed into the developing-bath mentioned hereinbefore, rinsed, soaped and rinsed once more.

In this manner beautiful light brown shades of an excellent fastness are obtained.

#### EXAMPLE 6.

##### Dyeing calico in pieces in reddish-brown shades.

100 gr. of a paste, containing 15% of the anilid of 2,3-hydroxynaphthoic acid, the nitrosamin-alkali-salt of 3-nitro-1,4-tolidin and free caustic soda solution, are stirred with

200 gr. of cold water and dissolved in further

500 gr. of water, then

20 gr. of the product, prepared from indigo according to the U. S. A. Letters Patent No. 1,448,251, dissolved in

180 gr. of water, are added and the whole is made up to

1000 gr.

The goods are impregnated upon a foulard-apparatus with this solution, dried, hung out for some hours and then passed into the developing-bath mentioned hereinbefore.

In this manner a beautiful reddish brown of an excellent fastness is obtained.

## EXAMPLE 7.

The unprepared goods are printed with the following printing color:

5 10 gr. of 4-hydroxynaphthalene-1-phenylketone are mixed with  
30 cc. of caustic soda solution of 34° Bé.,  
30 gr. of Turkey red oil and  
200 gr. of water, poured in  
10 500 gr. of neutral tragacanth thickening  
and  
10 gr. of the product, prepared from indigo according to the U. S. A. Letters Patent No. 1,448,251, dissolved in  
15 220 gr. of water, are added and the whole is made up to

1000 gr.

20 Then the goods are printed with a second printing-color:

10 gr. of 5-chloro-2-toluidin are dissolved with  
15 gr. of hydrochloric acid of 22° Bé. and  
25 100 gr. of boiling water,  
160 gr. of ice and after cooling down  
25 cc. of sodium nitrate 1:4 are added; the diazotization being complete, the mass is poured in  
30 500 gr. of neutral tragacanth thickening,  
25 gr. of sodium acetate and  
165 gr. of water are added and the whole is made up to

35 1000 gr.

The goods are dried and passed into the above mentioned developing-bath, rinsed, soaped and dried.

A chocolate-brown is obtained.

## EXAMPLE 8.

The unprepared goods are printed with:  
10 gr. of benzoyl-2, 3-aminonaphthol are mixed with

45 30 cc. of caustic soda solution of 34° Bé.,  
30 gr. of Turkey red oil and  
200 gr. of water, poured in  
500 gr. of neutral tragacanth thickening and

50 10 gr. of the product, prepared from indigo according to the U. S. A. Letters Patent No. 1,448,251, dissolved in

55 220 gr. of water, are added and the whole is made up to

1000 gr.

The goods are dried and printed once more with:

10 gr. of 4-nitro-1,2-anisidin are dissolved with  
15 gr. of hydrochloric acid of 22° Bé. and  
100 gr. of boiling water,  
160 gr. of ice and after cooling down  
25 cc. of soda nitrate 1:4 are added; the diazotization being complete, the mass is poured in  
500 gr. of neutral tragacanth thickening,  
25 gr. of sodium acetate and  
165 gr. of water are added and the whole is made up to

1000 gr.

The goods are dried and passed into the above mentioned developing-bath, rinsed, soaped and dried.

A dark reddish brown is obtained.

## EXAMPLE 9.

80

The goods are prepared with a solution of 12 gr. of 2,5-dichlorophenyl-3-methyl-5-pyrazolone in 15 cc. of caustic soda solution of 34° Bé. by addition of 10 gr. of Turkey red oil and 8 gr. of the products, prepared from indigo according to the U. S. A. Letters Patent No. 1,448,251, in the liter.

The goods are dried and printed with:  
16.5 gr. of 2,5-dichloroanilin are dissolved with

100 gr. of hot water and  
50 cc. of hydrochloric acid of 20° Bé.,  
200 gr. of ice and after cooling down  
8 gr. of sodium nitrite of a standard of 95%, dissolved in  
30 gr. of water, are added; the diazotization being complete the mass is poured in  
500 gr. of neutral tragacanth thickening,  
45 gr. of sodium acetate and  
59 gr. of water are added and the whole is made up to

100

105

1000 gr.

The goods are dried and passed into the above mentioned developing-bath, rinsed, soaped, rinsed and dried.

A green upon a blue ground is obtained.

## EXAMPLE 10.

The goods are prepared with a solution of 10 gr. of aceto-acetyl-anilin in 15 gr. of caustic soda solution of 34° Bé. by adding 10 gr. of Turkey red oil in the liter.

4

The goods are dried and printed with:  
 10 gr. of 5-nitro-1,2-toluidin are mixed  
 with  
 25 gr. of hot water and  
 5 gr. of sodium nitrite, poured in  
 350 gr. of water and  
 30 cc. of hydrochloric acid of 20° Bé.; the  
 diazotization being complete the  
 mass is stirred in  
 10 450 gr. of neutral tragacanth thickening,  
 70 gr. of sodium acetate 1:1 and  
 10 gr. of the product, prepared from in-  
 digo according to the U. S. A.  
 Letters Patent No. 1,488,251, dis-  
 solved in  
 50 gr. of water, are added and the whole  
 is made up to  
 1000 gr.

20 The goods are dried and passed into the  
 above mentioned developing-bath, rinsed,  
 soaped, rinsed and dried.  
 A yellowish green is obtained.

25 By using 10 gr. of the product, prepared  
 from dibromindigo according to the U. S. A.  
 Letters Patent No. 1,448,251, instead of the  
 above mentioned indigo derivative, a little  
 more yellowish shades of a greater clearness  
 are obtained.

#### EXAMPLE 11.

35 The goods are impregnated with a solution  
 of 10 gr. of acetoacetyl-para-anisidin in 15  
 cc. of caustic soda solution of 34° Bé. by  
 adding 10 gr. of Turkey red oil in the liter.  
 The goods are dried and printed with:

40 10 gr. of the product, prepared from indi-  
 go according to the U. S. A. Let-  
 ters Patent No. 1,448,251, dis-  
 solved in

45 490 gr. of water, poured in  
 500 gr. of neutral tragacanth thickening,  
 made up to

1000 gr.  
 The goods are dried and printed once  
 more with:

50 13 gr. of ortho-chloroanilin are dis-  
 solved with  
 30 gr. of hot water and  
 30 cc. of hydrochloric acid 20° Bé.,  
 55 140 gr. of cold water,  
 150 gr. of ice and after cooling down  
 7.5 gr. of sodium nitrite and  
 30 gr. of water are added; the diazota-  
 tion being complete the mass is  
 poured in  
 60 450 gr. of neutral tragacanth thickening,  
 50 cc. of sodium acetate 1:1 are added  
 and the whole is made up to

65 1000 gr.

The goods are dried, passed into the above 70  
 mentioned developing-bath, rinsed, soaped,  
 rinsed and dried.

Blue, green and yellow printing-effects on  
 a white ground are obtained.

#### EXAMPLE 12.

The cotton goods are prepared with the  
 following padding-solution and dried: 8 gr.  
 of meta-nitroanilid of 2,3-hydroxynaphthoic  
 acid, 10 cc. of caustic soda solution of 34° 80  
 Bé., 8 gr. of Turkey red oil, 1 liter.

The goods are then printed with the fol-  
 lowing printing-color:

10 gr. of meta-nitro-ortho-anisidin  
 $(OCH_3 : NH_2 : NO_2 = 1:2:4)$  85  
 are dissolved with

15 gr. of hydrochloric acid of 22° Bé. and  
 100 gr. of boiling water and  
 160 gr. of ice are added. After cooling 90  
 down while stirring

25 cc. of sodium nitrite 1:1 are added.  
 The diazotization being complete,  
 the mass is poured in

500 gr. of neutral tragacanth thickening, 95  
 neutralized with

25 gr. of sodium acetate and  
 20 gr. of the product, prepared from indi-  
 go according to the U. S. A. Let-  
 ters Patent No. 1,448,251, dis-  
 solved in

145 gr. of water, are added and the whole  
 is made up to

1000 gr.  
 The goods are dried, steamed for a short 105  
 while and passed into the above mentioned  
 developing-bath, rinsed, soaped and dried.

A dark violet of an excellent fastness is  
 obtained.

#### EXAMPLE 13.

The cotton goods are prepared with the  
 following solution and dried.

##### Padding-solution 1.

115 10 gr. of diacetoacetyl-ortho-tolidin, 12 cc.  
 of caustic soda solution of 34° Bé., 10 gr. of  
 Turkey red oil, 1 liter.

The goods are then padded with the fol-  
 lowing solution:

##### Padding-solution 2.

125 50 gr. of the diazo-salt of 2,5-dichloro-  
 anilin are dissolved in

300 gr. of water and  
 400 gr. of neutral tragacanth thickening,

120 10 gr. of the product, prepared from in-  
 digo according to the U. S. A.  
 Letters Patent No. 1,448,251, dis-  
 solved in

130 240 gr. of water, are added and the whole  
 is made up to

1000 gr.

The goods are dried, steamed for a short while and passed into the above mentioned developing-bath, rinsed, soaped, rinsed and dried.

5 A light green shade of an excellent fastness is obtained.

EXAMPLE 14.

The unprepared goods are printed with 10 the following printing-color and dried:

Printing-color 1.

10 gr. of meta-nitroanilid of 2,3 hydroxy-naphthoic acid,

15 12 cc. of caustic soda solution of 34° Bé, 10 gr. of Turkey red oil are dissolved in 200 gr. of boiling water and poured in 500 gr. of neutral tragacanth thickening.

After cooling down

20 10 gr. of the product, prepared from indigo according to the U. S. A. Letters Patent No. 1,448,251, dissolved in

25 258 gr. of water, are added and the whole is made up to

1000 gr.

The goods are printed once more with a second printing-color or padded with a corresponding solution.

Printing-color 2.

50 gr. of the diazo-salt of 2,5 dichloro-anilin are dissolved in

35 450 gr. of water and poured in 500 gr. of a neutral tragacanth thickening and the whole is made up to

1000 gr.

40 The goods are dried and passed into a lukewarm to boiling bath, containing 3 gr. of iron chloride, 1 gr. of bichromate, 25 gr. of sodium bisulfate, 1 liter, rinsed, soaped and dried.

45 A reddish brown of an excellent fastness is obtained.

EXAMPLE 15.

The unprepared goods are printed with the following printing-color:

50 Printing-color 1.

10 gr. of diacetoacetyl-ortho-tolidin,

12 cc. of caustic soda solution of 34° Bé,

55 10 gr. of Turkey red oil are dissolved in 200 gr. of boiling water and poured in 500 gr. of neutral tragacanth thickening.

After cooling down

60 10 gr. of the product, prepared from indigo according to the U. S. A. Letters Patent No. 1,448,251, dissolved in

258 gr. of water, are added and the whole is made to

65 1000 gr.

The goods are printed with a second printing-color or padded with a corresponding solution.

Printing-color 2.

70

10 gr. of meta-nitro-ortho-anisidin

(OCH<sub>3</sub>:NH<sub>2</sub>:NO<sub>2</sub>=1:2:4)

75

are dissolved with

15 gr. of hydrochloric acid of 22° Bé. and

100 gr. of boiling water,

165 gr. of cold water,

160 gr. of ice are added, after cooling 80 down

25 cc. of sodium nitrite 1:4, poured in 500 gr. of neutral tragacanth thickening,

and

25 gr. of sodium acetate are added and 85 the whole is made up to

1000 gr.

The goods are dried and passed into the 90 bath mentioned in Example 14, rinsed, soaped and dried.

A green of an excellent fastness is obtained.

By varying the proportions of mixtures 95 and the components thereof numerous further shades can be obtained.

In the same manner, as the ester-salt of the leuco-derivative of indigo, the corresponding derivatives of the halogenated indigos, thiocindigo and other vat dyestuffs 100 can be used. As suitable oxidizing agents we may mention: hydrogenperoxide, perborates, persulfates or chlorates, chromates and so on.

An appropriate oxidizing agent may also be added to the printing-colors. Then as developing-baths only accordingly diluted acids or solutions of salts, acting as acids, may be used. Certain features of the invention disclosed herein are claimed in another application filed by us in the United States Patent Office on June 24, 1925, Serial No. 39,377.

Now what we claim and desire to secure 115 by Letters Patent is the following:

1. A process of producing combined shades of azodyestuffs and vat dyestuffs on the vegetable fiber consisting in producing an azodyestuff on the fiber, an ester-salt of the leuco-compound of a vat dyestuff being present simultaneously, and in treating the fibers with oxidizing agents in an acid medium.

2. Materials dyed with a mixture of an azodyestuff and a vat dyestuff according to claim 1.

3. A process of producing combined shades of azodyestuffs and vat dyestuffs on 1.

the vegetable fiber consisting in impregnating the fiber with a mixture of an aromatic nitrosamin-alkali-salt and an alkali-salt of an azo-component and an ester-salt of the 5 leucocompound of a vat dyestuff and in developing the dyestuffs by treatment with oxidizing agents in an acid medium.

4. Materials dyed with a mixture of an

azodyestuff and a vat dyestuff according to claim 3.

In testimony, that we claim the foregoing as our invention, we have signed our names, this 29th day of November, 1924.

GUSTAV PETZOLD.  
HEINRICH RITTNER.